

Oct. 20, 1931.

T. H. FROST

1,827,872

FINE EDGED BLADE

Filed Nov. 14, 1930



Fig. 1.



Fig. 2.



Fig. 3.



Fig. 4.



Fig. 5.



Fig. 6.

INVENTOR.  
Thomas H. Frost  
by *W.M. Farrow, AIA*

## UNITED STATES PATENT OFFICE

THOMAS H. FROST, OF CAMBRIDGE, MASSACHUSETTS

## FINE EDGED BLADE

Application filed November 14, 1930. Serial No. 495,657.

This invention relates to fine edged blades of ferrous alloys which may be hardened by the process of nitriding. In one aspect it comprises a novel blade of such alloy characterized by a plated unnitrided body portion and a narrow unplated nitrided area in which the cutting edge is included. In another aspect it comprises an improved method of producing such blades.

10 An important field of use of my invention is in the production of safety razor blades of the thin flexible type which are adapted for use in holders wherein they are clamped for support. In my prior applications Ser. No. 455,366, filed May 24, 1930, and Ser. No. 494,591 filed November 10, 1930, I have disclosed safety razor blades with nitrided cutting edges and in still another aspect the present invention constitutes a development or 20 carrying forward of these earlier inventions.

The material I prefer to employ in the construction of the novel blade of my invention is a ferrous alloy containing a substantial amount of aluminum usually combined with 25 chromium or molybdenum or tungsten. An example of such alloy is the material commercially known as nitralloy and, while this is suitable for manufacture of fine-edged blades, any other ferrous alloy capable of being hardened by the process of nitriding may 30 be used, being selected in accordance with the requirements of the particular blade under construction.

When such metal is exposed to ammonia fumes under conditions of high temperature it becomes nitrided upon its exposed surfaces and an extremely hard brittle case is formed thereon which may extend slightly below the surface of the blank. Difficulty has been experienced heretofore in nitriding a flat blank 35 on account of the fact that expansion of the material takes place in the nitriding operation which tends to warp or distort it to an objectionable extent, moreover blades nitrided throughout their area are too brittle for practical purposes. This is particularly true of such an article as a flexible safety razor blade which is commonly maintained in a position of pronounced curvature when in 40 use and must therefore be capable of with-

standing appreciable bending. A razor blade of completely nitrided material is likely to shatter when bent between the fingers and so become a menace to the user.

I have discovered that if the nitrided area 55 is confined to a narrow zone including little more than the bevelled portion of the blank or the vertex of the cutting edge then the blade as a whole, on account of its softer body portion, is rendered durable and capable of 60 such flexing as is commonly imposed upon safety razor blades. While the actual cutting edge of such a blade is extremely hard and brittle the more flexible, tougher body of the blade offsets the fragility of its cutting 65 edge and supports the same while being positioned or subject to use. I have discovered that an improved blade of these desirable characteristics may be produced by plating the body of the blank with a metal which is 70 impervious to ammonia fumes and then removing the plating from the margin of the blank in the narrow zone included in the cutting edge so as to expose the ferrous alloy 75 of the blank in this restricted area only. The 75 nitriding operation is then carried out upon the blank thus prepared with the result that it is nitrided and hardened only in the narrow marginal zone or zones from which the plating has been removed.

Preferably, and as herein shown, the method of my invention is characterized by simultaneously removing the plating in a narrow zone and partially forming a cutting edge upon the blank. This can be conveniently done by rough bevelling the edge of the blank and thus in a single operation two important functions are achieved, i. e.: the exposure of the ferrous alloy in the desired restricted area and the partial formation of 90 the cutting edge. After the nitriding operation the blade may be completed by further grinding or sharpening operations upon its rough bevelled and nitrided edge.

An important feature of a blade produced 95 as above outlined resides in the fact that it is thereby rendered rust-resistant throughout. This is because the plated surfaces of the blade upon the unnitrided portions thereof are protected by the plating itself which may 100

be of a non-ferrous, non-corrosive metal such for example as silver, copper, or tin, whereas the nitriding operation upon the exposed and unplated portions of the blade imparts to them all the rust-resistant properties of a high chromium steel. The latter property of nitr alloy and similar ferrous alloys has been recognized heretofore but this characteristic has not been heretofore utilized in the construction of fine-edged blades which are rust-resistant throughout. This feature is of extreme importance as applied to safety razor blades which are frequently moistened and imperfectly or hastily dried.

Another advantage incident to a blade of this character arises from the ornamental and attractive finish which the plating imparts to the blade. For example, a thin plating of silver is adequate to protect the body of the blade from the nitriding action and the silver-plated surface which results in the finished blade is extremely attractive and ornamental as a finish. Therefore, in carrying out the method of my invention, the single step of plating the blank is useful both in defining the unnitrided portions of the blade and in supplying a superior finish.

Still another advantage of the present invention resides in the fact that it can be applied to the manufacture of blades in strip form. Under such conditions the contour of the blades or of the blade blanks may be outlined in strip stock of a nitridable ferrous alloy. The strip may then be plated and subsequently rough-ground in strip form which, from a manufacturing standpoint, is an advantageous manner of carrying out these steps. The plated and rough ground blanks may then be nitrided either in the strip or as separated into individual blanks.

These and other features of my invention will be best understood and appreciated from the following description of a preferred manner of applying it to the manufacture of safety razor blades as illustrated in the accompanying drawings, in which:

Fig. 1 is a view in perspective of strip metal in which the blades have been outlined.

Fig. 2 is a similar view of the plated strip.

Fig. 3 is a similar view of the plated strip after the rough grinding step has been carried out.

Fig. 4 is a view in perspective of a stack of blanks ready for the nitriding step.

Fig. 5 is a sectional view on the line 5—5 of Fig. 4, and

Fig. 6 is a view in perspective of a finished blade.

In manufacturing safety razor blades by the method of my invention the blanks or blade blanks 10 are first outlined in strip-form. As shown in Fig. 1 this may be done by punching or dieing out suitable notches and perforations in a continuous strip or

ribbon of nitr alloy or other ferrous nitridable alloy which may be procured, rolled to the desired thickness. As herein shown each blade blank is provided with an internal aperture 12 in the shape of a slot intersecting spaced recesses and with cut-out portions which forms corner notches 14 to relieve the finished blade of corner-cap pressure. The strip may be scored or otherwise marked to set off one blank from the next but the step of outlining the blades and the ensuing steps of the method are carried out with the material in strip form.

The material employed for the production of the blank may advantageously be of either of the following analyses:

| Element    | Analysis (A) | Analysis (B) |
|------------|--------------|--------------|
| Carbon     | .36          | .23          |
| Manganese  | .51          | .51          |
| Silicon    | .27          | .20          |
| Aluminum   | 1.23         | 1.24         |
| Chromium   | 1.49         | 1.58         |
| Sulphur    | .010         | .011         |
| Phosphorus | .013         | .011         |
| Molybdenum | .18          | .20          |

The analyses above set forth are typical of a satisfactory nitr alloy material for the manufacture of fine edged blades but nitr alloy of other similar analyses may be success- 95 fully used.

The next step in carrying out the method of my invention consists in plating or coating the blade strip with a non-ferrous metal. I have found that tin, copper, silver nickel, 100 chromium and possibly other metals are suitable for this coating, and while any metal which is impervious to ammonia fumes would be satisfactory, I prefer to employ a silver-plating partly on account of the superior finish which is derived therefrom in the finished blades. In electro-plating the blade strip the entire surface of the strip is coated together with its exterior marginal edges and the interior edges of the aperture 110 12.

The next step consists in removing the plating from the narrow marginal zone of the strip in which the cutting edge is to be formed and this may be effected to best advantage by rough grinding the edges of the strip to form the bevel 16. This step as already noted not only removes the protective plating accurately in the defined area which is to be nitrided but also partially forms a cutting edge of the blade. In some cases, other than in the manufacture of safety razor blades, the rough grinding step may be all that is required to produce an edge of sufficient keenness for the intended purpose of the blade.

Having completed the grinding operation upon the blade strip the latter is separated into individual blanks by being broken on the scored lines and the rough-bevelled 120 125

- blanks are stacked flatwise and secured in such position. Any convenient number of blanks may be stacked and preferably these are clamped as suggested in Fig. 4 between a thick bottom plate 20 and a thick top plate 22 secured together by clamping bolts 34 which pass through the plates and through the apertures of the blade blanks. Having arranged the blanks in stack form as above outlined with or without the addition of spacing shims the stack is placed in a furnace and subjected to the action of ammonia gas for a predetermined interval of time and at a proper temperature for the nitriding requirements of the blade. Satisfactory blades may be produced from nitrallloy of the analyses above set forth by subjecting the stack to a temperature of about 900° F. to 950° F. or thereabouts for a period of two hours.
- Under these circumstances the exposed bevel edges of the blades will have a hard nitrided case formed thereon but nowhere else, while the blade as a whole will be maintained in flat condition in the stack. The case may extend entirely through the material of the bevel or it may extend merely a few thousandths of an inch below the surface thereof but in any case the vertex of the blade is completely nitrided.
- After the conclusion of the nitriding step the stack is removed from the furnace and allowed to cool thereupon the clamping bolts 24 may be released and the blades separated. The hardened nitrided case permits the rough bevel 16 of the blank to be finish ground, honed and stropped to produce the smooth bevel 17 of the finished blade 11 shown in Fig. 6. The silver plated surface of the blade presents at all times an attractive finish and may be rendered brilliant by a slight buffing operation. As already intimated the elongated narrow nitrided zone defined by the bevel 17 in the finished blade is of extreme hardness and although it is also brittle it is carried and distributed along the unnitrided soft and flexible body of the blade in such a manner that, as a complete article, the blade affords satisfactory service.
- Having thus described my invention what I claim as new and wish to secure by Letters Patent of the United States is—
1. A fine edged blade of a nitridable alloy, bevelled to form a cutting edge, nitrided only in a narrow zone defined by the bevel and plated throughout the remainder of its surface.
  2. A fine edged blade of a nitridable alloy, having a plated body limited in its area by a bevelled edge portion and being nitrided in such bevelled portion only.
  3. A fine edged blade of a nitridable alloy, having supplementary plated and nitrided areas, whereby the whole surface of the blade is rendered rust-resistant.
  4. A fine edged blade of a nitridable alloy,
- having flat plated areas and supplementary bevelled areas which are nitrided, whereby the whole surface of the blade is rendered rust-resistant.
5. A fine edged blade of a nitridable alloy, 70 bevelled to form a cutting edge, having a non-ferrous plating upon its body and being nitrided in a narrow zone which is substantially coextensive with its bevelled cutting edge.
6. A fine edged blade of a nitridable alloy, internally apertured to receive blade positioning means and being plated upon its surface and the marginal edges of its aperture, and having an unplated bevelled and nitrided 80 cutting edge.
7. The method of making fine edged blades, which consists in producing a flat blank of a nitridable ferrous alloy plated upon its surfaces except in a narrow marginal portion 85 thereof, nitriding said marginal portion and reducing it to a cutting edge.
8. The method of making fine edged blades, which consists in producing a blank of a nitridable ferrous alloy, forming an ornamental and protective plating on the surfaces thereof, beveling a marginal portion of the blank to remove the plating in a narrow zone, and nitriding the portion of the blank thus exposed.
9. The method of making fine edged blades, which consists in defining the outline of the blade in sheet stock of nitridable ferrous alloy, plating the entire area so defined, removing the plating in a narrow marginal zone and reducing the thickness of the blank in the same zone, nitriding the stock thus exposed, and then finish grinding to produce a cutting edge in nitrided stock.
10. The method of making fine edged blades, which consists in producing a blank having an internal aperture from a nitridable ferrous alloy, plating the surface of the blank including the marginal edges of its aperture, beveling an outer edge of the blank to remove the plating, and then nitriding the ferrous alloy thus exposed.
11. The method of making fine edged blades, which consists in producing a blade blank in ferrous nitridable alloy, rendering the entire blank rust-resistant by plating the surface thereof and nitriding the outer edge, and forming a cutting edge in the nitrided portion of the blank.
12. The method of making fine edged blades, which consists in outlining the blade blanks in a strip of nitridable ferrous alloy, plating the strip, rough grinding the margin of the plated strip to remove the plating and partially form a cutting edge, separating the strip into individual blanks, nitriding the bevelled portions of the blanks, and finish grinding the nitrided portions to complete the blades.
13. A fine edged blade of a nitridable fer-

rous alloy, having a silver plated body limited in its area by a bevelled edge portion and being nitrided in such bevelled portion only.

5 14. A fine edged blade of a nitridable ferrous alloy, bevelled to form a cutting edge, having a nickel plating upon its body and being nitrided in a narrow zone which is substantially coextensive with its bevelled cutting edge.

10 Signed at Boston, Massachusetts, this 12th day of November, 1930.

THOMAS H. FROST.

15

20

25

30

35

40

45

50

55

60